

Oct. 16, 1928.

W. H. DROEGE

1,688,138

ARTIFICIAL PLANK

Filed July 23, 1925

Fig. 1.



Fig. 2.

Fig. 3.



Fig. 5.



Fig. 6.

INVENTOR.

W. H. Droege

BY

Elwin M. Huber

ATTORNEY.

Patented Oct. 16, 1928.

## UNITED STATES PATENT OFFICE.

WILLIAM H. DROEGE, OF FORT WAYNE, INDIANA.

## ARTIFICIAL PLANK.

Application filed July 23, 1925. Serial No. 45,641.

The invention relates to artificial planks adapted primarily for railroad crossings at highways.

The object of the invention is to provide a plank which may be made and laid at a minimum of cost and which will form a highly efficient crossing material of long life.

The invention consists in a plank formed of selected materials in such manner that each plank fits into and supports another.

I have found that a plank formed of bitumen, silica or limestone dust, steel or cast iron dust and finely divided gravel, stone or quartz is of long life and admirably fitted for railroad crossing uses. I prefer to use refined asphalt bitumen and in forming the plank I mix together 16 to 25% of silica dust or limestone dust and 54 to 71% of a graded sand, gravel, stone or quartz and 5 to 10% of powdered steel or iron and heat the mixture to a temperature of not less than 325° Fahr-enheit and while the mixture is hot I insert 8 to 11% of the bitumen, thoroughly mixing it with the aggregate to coat each particle thereof. The mixture is then inserted into a mold, a suitable reinforcing member is inserted into the mass and a pressure of approximately 1500 pounds per square inch is then applied to compress the mass and cause it to assume the shape of the mold.

It is desirable that the bitumen shall have a specific gravity of not less than 1.02; that the silica or limestone shall be not larger than such as will pass through a 200 mesh screen and the gravel, stone or quartz should be of such size as to form an almost voidless composition after compression.

The pulverized steel or iron lessens the possibility of the finer materials loosening between the grains of silica or limestone dust or the particles of gravel, stone or quartz, and it materially increases the resistance of the plank to traffic and shock.

When the compressed mass is removed from the mold and has cooled it has the form of the mold and when laid at a grade crossing a surface is presented which resists wear by the traffic. The plank is also fire proof. No spiking of the plank to the ties is necessary and it is easy to lay and take up.

In the drawings Figure 1 is a perspective view of the finished plank; Fig. 2 a plan view of the plank; Fig. 3 a longitudinal cross-section on line 3-3 of Fig. 2; Fig. 4

55 a transverse cross-section on line 4-4 of

Fig. 2; Fig. 5 a plan view of a railway crossing having the invention applied thereto and Fig. 6 a cross-section on line 6-6 of Fig. 5.

In the drawings the fabricated plank 1 is provided with an end rib 2 and a groove 3 at its opposite end for interlocking end-wise with other similar planks. A rib 4 is formed on one side of the plank and a groove 5 is formed in the opposite side. The reinforcement comprises a rod 6 from the opposite sides of which project the lugs 7. This reinforcement extends substantially from end to end of the plank and the lugs thereof project toward the opposite sides of the plank preferably at an angle to the longitudinal axis of the rod. The reinforcement therefore reinforces the central portion of the plank and causes the same to have a maximum of strength and rigidity.

The ribs on one plank fit into the grooves of other planks so that when a number of these planks are laid at a railway crossing they are interlocked and will remain in position. Their weight is sufficient to hold them in place but they may be secured in place in any suitable manner when it is desirable to do so. The side ribs on the planks adjacent one rail 8 of the track may project under the tread of the rail and thereby further lock the planks in place and this without interfering with the travel of the vehicle wheels on the rail. The planks adjacent the opposite rails 9 of the track could be made with ribs 5a on their opposite sides so that the planks may be interlocked with their neighbors and with the rails.

The plank may be used for various purposes, hence it is not limited in its use at grade crossings. The interlocking elements may also be of various forms, the form illustrated being one such only.

In the claim I shall use the term "gravel" intending thereby to include sand, stone and quartz, since finely divided gravel is in reality sand.

What I claim is:

A plank composed of a mixture of 8 to 11% of bitumen, 16 to 25% of stone dust, 54 to 71% of finely divided gravel and 5 to 10% of powdered iron.

In witness whereof I have hereunto set my hand this 21st day of July, 1925.

WILLIAM H. DROEGE.